

E. E. SLICK.

METHOD OF FORMING FLANGED METAL WHEELS.

APPLICATION FILED NOV. 14, 1908. RENEWED MAY 18, 1910.

965,041.

Patented July 19, 1910.

3 SHEETS—SHEET 1.

*Fig. 1.*



*Fig. 2.*



*Fig. 3.*



*Fig. 4.*



*Fig. 5.*



WITNESSES

*R. S. Little*  
*G. L. Winters*

INVENTOR

*E. E. Slick*  
by *Barclay Bynes* *Scoville*  
*his attorney*

E. E. SLICK.

METHOD OF FORMING FLANGED METAL WHEELS.

APPLICATION FILED NOV. 14, 1908. RENEWED MAY 18, 1910.

965,041.

Patented July 19, 1910.

3 SHEETS—SHEET 2.

Fig. 6.



Fig. 7.



Fig. 8.



WITNESSES

R. S. Little  
J. G. McIntire.

INVENTOR

E. E. Slick  
G. Wallace Byers & Sonule,  
his atty.

965,041.

E. E. SLICK.

METHOD OF FORMING FLANGED METAL WHEELS.

APPLICATION FILED NOV. 14, 1908. RENEWED MAY 18, 1910.

Patented July 19, 1910.

3 SHEETS—SHEET 3.

*Fig. 9.*



*Fig. 10.*



*Fig. 11.*



WITNESSES

R. D. Little.  
G. L. Winters.

INVENTOR

E. E. Slick  
by *Patent Office, New York, N.Y.*  
*his attorney*

# UNITED STATES PATENT OFFICE.

EDWIN E. SLICK, OF PITTSBURG, PENNSYLVANIA.

## METHOD OF FORMING FLANGED METAL WHEELS.

965,041.

Specification of Letters Patent. Patented July 19, 1910.

Application filed November 14, 1908, Serial No. 462,608. Renewed May 18, 1910. Serial No. 562,067.

To all whom it may concern:

Be it known that I, EDWIN E. SLICK, of Pittsburg, Allegheny county, Pennsylvania, have invented a new and useful Method of

5 Forming Flanged Metal Wheels, of which the following is a full, clear, and exact description, reference being had to the accompanying drawings, forming part of this specification, in which—

10 Figure 1 is a plan view of a cast ingot, as made in accordance with my invention; Fig. 2 is a similar view showing the ingot of Fig. 1 as reduced and formed in the first step of my improved method; Fig. 3 is a 15 plan view showing the manner in which the ingot of Figs. 1 and 2 is cut into wheel blanks in the next step in the method forming my invention; Figs. 4 and 5 are sectional views showing reciprocating forging dies 20 adapted to form the wheel blanks of Fig. 3 into flanged wheels in accordance with my invention; Figs. 6, 7 and 8 are sectional views showing rocking or rotating dies arranged with the axes of the opposing dies 25 at an angle to each other and adapted to carry out the forging operation in forming the wheel blanks of Fig. 3 into flanged wheels in accordance with my invention; and Figs. 9, 10 and 11 are sectional views 30 similar to Fig. 4 showing the flow of metal in successive steps of the forging operation in forming the blank shown dotted in Fig. 4 into the shape shown in section in Fig. 4, the blank shown dotted in Fig. 4 being the same as the blank shown in full lines in 35 Fig. 9.

My invention relates to the manufacture of wrought metal wheels, in which a hub is joined by a continuous web to a rim portion, and it particularly relates to wheels formed integral and having hub, web and flanged tread or rim portions.

The object of the invention is to provide a novel and effective method of forming such wheels, including a series of related steps beginning with the casting operation and ending with the forged wheel, by the use of which strong and durable wheels are obtained having marked and well defined 45 characteristics of structure not present in such forged metal wheels as made heretofore.

The invention is also designed to provide an improved method of forming wheels in 50 which the number of operations is reduced, the expense of making the wheels is lessened,

and in which the resulting product is cheapened while wheels of an improved quality are obtained.

The invention consists in an improved 60 method of making flanged wheels of wrought metal, including the casting of the multiple length blank, the severing of the cast blank transversely into single wheel blanks, and the forging operations, by a 65 series of novel steps by which a wheel is produced in which the grain or fiber of the metal is not crossed by any point on the wearing surfaces of the finished wheel, and by which the grain or fiber of the metal extends in the same general direction axially 70 outward at all points in the periphery of the finished wheel.

The invention also consists in forming a 75 wrought blank with its axially central portion formed from the axially central portion of the cast blank and then displacing metal intermediate of the hub and edge of the blank into the flange of the wheel.

The invention also consists in making 80 forged metal wheels having a flange portion formed of metal displaced from the body of the blank between the axial center and the periphery or marginal edge of the blank and having a tread portion whose 85 outer side or edge portion is formed of metal displaced from the periphery or marginal edge of the blank or ingot.

The invention further consists in severing 90 a cast ingot transversely into wheel blanks and forging the severed blanks into wheels having their wearing surfaces or periphery formed from the cut surface of the severed blank.

The invention still further consists in 95 the method of forming wrought metal wheels in which the blanks are forged into wheels and surplus metal in the blank is displaced by the forging operation and is caused to form a peripheral fin which extends outwardly from the wheel at an angle 100 to a transverse center line and in this manner enables blanks of varying sizes and weights to be forged into wheels of a practically constant thickness and weight.

In the drawings, 2 represents a multiple 105 length cast ingot having a circular or polygonal cross-section, and 3 is the ingot after having been reduced transversely in area by rolling or forging this operation densifying 110 the metal from its periphery inward toward its axial center and changing its cast granu-

lar structure into a fibrous structure. The blank 3 is then severed transversely by shearing, sawing, or in any other desired manner, into cylindrical cheese shaped wheel blanks 4 of the desired weight and thickness. Preferably the cut blank is at least as thick as the thickness through the hub of the finished wheel. The cut wheel blanks are reheated, and are then forged into finished 10 wheels by means of suitable forming dies, either reciprocating dies, rotary dies, or rocking dies having their axes at an angle to each other being employed to carry out the forming operations.

15 In carrying out the forging operation by means of reciprocating dies, such as are shown in Figs. 4 and 5, the cut blank is placed between the dies 5 and 6 of Fig. 4 in the position shown by dotted lines therein. 20 The movable die is then reciprocated to press or force the blank into the shape shown by 7 in Fig. 4. The partly formed blank 7 is then preferably removed, to a second set of reciprocating forging dies 8 and 9 having 25 die cavities as shown in Fig. 5, and the blank 7 is then further forged, to complete the wheel 10. In Fig. 9 the blank shown in full lines is pressed into the form shown in dotted lines in the first stage of the forging 30 operation and on continuing the forging operation in these dies the shape is further changed from that shown dotted in Fig. 9 into that shown dotted in Fig. 10; by continuing the movement of the dies toward 35 each other the shape shown dotted in Fig. 10 is finally formed into that shown in dotted lines in Fig. 11, which is the same shape as that shown in section in Fig. 4.

It will be noted that in the forging operation 40 in the first set of dies 5 and 6, the blank is dished so as to cause what was the peripheral surface of the severed blank to form the outer surface of the tread of the wheel, and that in the succeeding forging operation 45 between the dies 8 and 9, the flange and the wearing surface of the tread is formed from metal which is displaced from its original location in the sheared or cut surface of the blank at a point between the peripheral edge and the axial center of the blank.

In carrying out the operations of forging the blanks by means of rotary or rocking dies having their axes at an angle to each other, as shown in Figs. 6, 7 and 8, the blank 55 7<sup>a</sup> is first reduced in thickness and is dished between rocking dies 11 and 12 having a contour preferably as shown therein, the cut blank being shown in dotted lines and the blank as dished in these dies being shown 60 in section. The partly formed blank 7<sup>a</sup> is then preferably removed to a second set of dies 13 and 14, in which the blank is further reduced and the forging operation is finished, the beginning of the second forging 65 operation being shown in Fig. 7, and the

completion of this forging operation being shown in Fig. 8, the dies in Figs. 7 and 8 being of similar shape. In the first set of dies 11 and 12 the blank 7<sup>a</sup> is dished into approximately the shape shown, and in the 70 next forging step the flange and tread are formed of displaced metal originally located between the periphery and axial center of the cut blank. The wearing surface of the flange and tread is in this way formed from 75 metal originally in the cut surface of the severed blank, the peripheral surface of the severed blank being displaced so as to form the outer edge of the tread of the finished wheel. This is of great advantage, as the 80 peripheral surface is liable to have surface defects which are in this way removed from the wearing surfaces of the wheel.

In forming the cut blanks from the ingot, the blanks may vary slightly in thickness 85 and weight, and should a slight amount of excess metal be present in the blank, by arranging the dies in the peculiar manner shown in the drawings, any such excess metal in the blanks will be rolled outwardly 90 and will form a fin on the peripheral edge portion of the flange of the wheel, the sides of the fin being parallel to or being at an angle other than a right angle to the axis of the blank. By these means I am enabled 95 to finish wheels to a certain thickness and weight from blanks having a varying weight or thickness, the thin fin formed by reason of such excess weight being formed in such position on the wheel that it does not retard 100 the rolling operation and prevent the dies being brought into their closed position.

While I have shown two sets of reciprocating dies and two sets of rotary or rocking dies having their axes at an angle to each other for forming the wheel by forging, but one set of dies may be employed to perform the forging operation, in such case the dies having die cavities similar to those shown in Figs. 5 or 8.

The advantages of my invention will be appreciated by those skilled in the art. By my peculiar method of forming the ingot, severing the ingot into blanks, and then forging the wheels by the steps as described, 115 I am enabled to produce rolled flanged wheels having a fibrous structure which does not cross at any point the periphery of the finished wheel, and in which the grain or fiber in the finished wheel bears the 120 same relation to its axis at all points around the axis. This is of particular value as it insures the tread portion of the wheels wearing regularly, and very largely prevents the formation of false flanges and flat spots on 125 such wheels.

The peculiar series of steps of manipulating the blank enables the forming of wheels having integral flange and tread portions in which the wearing surfaces of the flange and 130

tread are formed from metal in the sheared or cut surface of the severed blanks, and displaces the metal in the periphery of the cut blanks to the outer edge of the tread portion 5 of the wheel, and the number of steps necessary to form the wheels is reduced, the cost of such wheels being lessened thereby.

While in Figs. 4 and 5, I show the hub of the wheels solid, and Figs. 6, 7 and 8, the 10 hub of the wheel punched, the wheels may be punched either at the beginning of the forging operation or after the forging operation has been completed, or the blanks may be punched during an intermediate 15 stage of the forging operation, or simultaneously therewith, as is desired.

Changes in the arrangement and in the construction of the dies may be made without departing from my invention. The ingot 20 may be formed with a cylindrical or polygonal cross-section, forming approximately a circular shape, and may be of any desired length. The manner in which the cast ingot is reduced in cross-sectional area 25 and is severed into blanks, and the thickness of the blanks, may be varied, the number of forging steps in forming the wheels may be changed, and other modifications 30 may be made within the scope of the claims.

I claim:—

1. The method of forming wheels, consisting in taking an ingot, reducing its cross sectional area, severing transversely therefrom a blank having its axis extending in the same direction relative to the metal of 35 the blank that the axis of the ingot extended relative to the same metal, then forcing

metal intermediate the periphery and axial center outwardly into the rim portion of the wheel.

2. The method of forming wheels, consisting in taking an ingot, severing transversely therefrom a blank having its axis extending in the same direction relative to the metal of the blank that the axis of the ingot extended relative to the same metal, then forcing 40 metal intermediate the periphery and axial center outwardly into the rim portion of the wheel.

3. The method of forming wheels, consisting in taking an ingot, reducing its cross sectional area, severing transversely therefrom a blank having its axis extending in the same direction relative to the metal of the blank that the axis of the ingot extended relative to the same metal, then forcing 45 metal intermediate the periphery and axial center outwardly into the rim portion of the wheel.

4. The method of forming wheels, consisting in taking an ingot, severing transversely therefrom a blank having its axis extending in the same direction relative to the metal of the blank that the axis of the ingot extended relative to the same metal, then forcing 50 metal intermediate the periphery and axial center outwardly into the rim portion of the wheel.

In testimony whereof, I have hereunto set my hand.

EDWIN E. SLICK.

Witnesses:

R. D. LITTLE,  
H. M. CORWIN.